



US005286592A

**United States Patent [19]****Johnston et al.****[11] Patent Number: 5,286,592****[45] Date of Patent: Feb. 15, 1994****[54] ELECTROSTATOGRAPHIC TONER  
CONTAINING CYAN PIGMENT****[75] Inventors: Brian H. Johnston; Thomas H.  
Whiteades, both of Rochester, N.Y.****[73] Assignee: Eastman Kodak Company,  
Rochester, N.Y.****[21] Appl. No.: 888,697****[22] Filed: May 27, 1992****[51] Int. Cl.<sup>5</sup> G03G 9/09****[52] U.S. Cl. 430/106, 430/109,  
430/111****[58] Field of Search 430/106, 109, 45, 241,  
430/225, 111; 546/5, 6, 7****[56] References Cited****U.S. PATENT DOCUMENTS**

- Re. 31,072 11/1982 Tadwin et al. 430/99  
4,183,755 1/1980 Chapman et al. 430/213  
4,358,404 11/1982 Chapman et al. 260/156  
4,419,435 12/1983 Reczek et al. 430/223  
4,476,207 10/1984 Reczek et al. 430/17  
4,521,506 6/1985 Stolzenburg et al. 430/241

4,563,409 1/1986 Suzuki et al. 430/106  
4,833,060 5/1989 Nair et al. 430/137  
4,965,131 10/1990 Nair et al. 428/407

**FOREIGN PATENT DOCUMENTS**

62-147465 7/1987 Japan  
253759 10/1989 Japan

*Primary Examiner*—Marion E. McCamish  
*Assistant Examiner*—Rosemary Ashton  
*Attorney, Agent, or Firm*—Willard G. Montgomery

**[57] ABSTRACT**

Electrostatographic toner materials containing a cyan pigment which is a metal coordination complex of a substituted 6-heterocycloazo-3-pyridinol compound are disclosed. These pigments are formulated with fusible polymeric binders to provide a toner which exhibits excellent triboelectric properties and improved cyan color and hue when utilized in the electrostatographic process to produce colored electrophotographic images.

**18 Claims, No Drawings**

**ELECTROSTATOGRAPHIC TONER CONTAINING CYAN PIGMENT**

**CROSS REFERENCE TO RELATED PATENT APPLICATIONS**

This patent application is related to U.S. patent application Ser. No. 07/888,698 (entitled "Electrostatographic Toner Containing Magenta Pigment") and U.S. patent application Ser. No. 07/888,696 (entitled "Electrostatographic Toner Containing Yellow Pigment") which are both being filed concurrently with the present application and which both have common inventorship and a common assignee with the present patent application.

**FIELD OF THE INVENTION**

This invention relates to novel toner particles containing cyan pigments, their method of preparation and the use of these materials as developer components in the preparation of colored electrophotographic images.

**BACKGROUND OF THE INVENTION**

In the electrophotographic process, an image comprising an electrostatic field pattern, usually of non-uniform strength (also referred to as an electrostatic latent image), is formed on an insulative surface of an electrostatographic element by any of various methods. For example, the electrostatic latent image may be formed electrophotographically (i.e., by imagewise photo-induced dissipation of the strength of portions of an electrostatic field of uniform strength previously formed on a surface of an electrophotographic element comprising a photoconductive layer and an electrically conductive substrate), or it may be formed by dielectric recording (i.e., by direct electrical formation of an electrostatic field pattern on a surface of a dielectric material). Typically, the electrostatic latent image is then developed into a visible image by contacting the latent image with an electrostatographic developer. If desired, the latent image can be transferred to another surface before development.

One well known type of electrostatographic developer comprises a dry mixture of toner particles and carrier particles. Developers of this type are commonly employed in well-known electrostatographic development processes such as cascade development and magnetic brush development. The particles in such developers are formulated such that the toner particles and carrier particles occupy different positions in the triboelectrical continuum, so that when they contact each other during mixing to form the developer, they become triboelectrically charged. The toner particles thus acquire a charge of one polarity and the carrier particles acquire a charge of the opposite polarity. These opposite charges attract each other such that the toner particles cling to the surfaces of the carrier particles. When the developer is brought into developing, e.g., contact relation, with the latent electrostatic image, the electrostatic forces of the latent image (sometimes in combination with an additional applied field) attract the toner particles, and the toner particles are pulled away from the carrier particles and become electrostatically attached imagewise to the latent image-bearing surface. The resultant toner image can then be fixed in place on the surface by application of heat or other known meth-

ods or can be transferred to another surface to which it then can be similarly fixed.

A more recent development of the electrostatographic process is its application for the production of colored images. These systems are based on trichromatic color synthesis such as produced by subtractive color formation wherein at least three separate color separation images are formed and the combined images brought into register with each other to form a colored reproduction of a full colored original.

In accordance with such a process, a photoconductor having a uniformly charged photoconductive surface (photoreceptor) capable of forming an electrostatic latent image is exposed through a green filter to an imagewise projection of a color image to form an electrostatic latent image on the photoreceptor. This electrostatic latent image is then developed with the complementary magenta color toner to form a magenta colored image corresponding to said electrostatic latent image, and transferred in register to an image receiving member. The photoreceptor is then electrostatically charged uniformly in the dark and exposed through a red filter to an imagewise projection of a color image in register with said magenta developed image to form a second electrostatic latent image, which second image is developed with the complementary cyan color toner and likewise transferred in register. The photoconductor is again electrostatically uniformly charged in the dark and then exposed through a blue filter to an imagewise projection of a color image in register with said magenta and cyan developed images to form a third electrostatic latent image which is then developed with the complementary yellow toner and again transferred in register. The sequence of exposures through colored filters in this multiple development process may be performed in any suitable sequence other than the green, red and blue mentioned.

This combination of three color toner images is generally made on a copy sheet transfer member such as paper or clear plastic to which the toner images are permanently affixed. One of the most common techniques for fixing these toner images to the copy sheet comprises employing a fusible resin toner which includes a colorant, and heat fixing the toner images to the copy sheet. Images may also be fixed by other techniques such as for example, subjecting them to a solvent vapor.

In most regions of the transfer member, the transferred layers are coated one on top of the other, the first layer being the magenta layer, the second being the cyan layer and the third being the yellow layer. Each subtractive color transmits two thirds of the spectrum and absorbs one third. The combination of cyan, magenta and yellow layers appears black, while the combination of magenta and yellow layers appears red, the combination of magenta and cyan layers appears blue, and the combination of yellow and cyan layers appears green. Images of enhanced contrast may also be prepared using a fourth black-colored toner in combination with the cyan, magenta and yellow toners described above.

In the color process, a colorant and resin combination used to make the toner must meet a number of stringent requirements. First, the formulated colorant must be of the correct color and hue within its spectral band width with minimal response in other bands so that it works together with complementary colorants to produce faithful color reproductions. Second, a colorant and

resin combination must be selected such that the toner possesses the appropriate triboelectric properties which will enable it to function and continue to function in an electrophotographic imaging mode. It is a function of the toner-carrier combination or developer package in a given development system, for example cascade, to assume a triboelectric relationship such that the toner will be carried with the carrier during the development cycle by electrostatic attraction and then be selectively deposited charge-wise on the electrostatic latent image which has a greater affinity for the toner electrostatically than does the carrier particle. In addition to the very significant triboelectric properties that a developer must possess and maintain during the development cycle, the toner must not only possess the appropriate color, but must also continue to function under machine conditions which expose the developer to impaction, humidity and oxygen among other undesirable factors. Third, the colorant used in formulating colored toner must be sufficiently color stable such that toner material of the requisite particle size, i.e., preferably from about 2 to about 20 microns, can be prepared without any significant diminution of color properties of the toner such as spectral response, color mixing characteristics and transparency. Finally, toners containing such colorants must also exhibit good transfer characteristics and the colorants preferably should have good heat and light stability.

Quite clearly, requirements must be met for the provision of colored toner materials capable of reproducing faithful electrostatographic reproductions of colored originals which are more stringent than the fact that a particular pigment used to produce the toner may be of a magenta, cyan or yellow color.

#### SUMMARY OF THE INVENTION

The present invention is directed to novel electrostatographic toner and developer compositions containing a cyan pigment which is based on a 1:1 coordination complex of an azo dye and a polyvalent metal ion, and having the structure of Formula 1:



or a 2:1 coordination complex of an azo dye and a polyvalent metal ion and having the structure of Formula 2:



In the above formula:

20 R is selected from the group consisting of OH and NH<sub>2</sub>,

25 R<sup>1</sup> is selected from the group consisting of hydrogen and C<sub>1</sub> to C<sub>6</sub> alkyl,

30 R<sup>2</sup> is selected from the group consisting of hydrogen, an alkyl group having from 1 to about 6 carbon atoms, acyl, aryl, aralkyl, alkylsulfonyl, amino, alkoxy, halogen, morpholino, phenylsulfamoyl, sulfonamido, sulfamoyl, carboxy and sulfo and hydrolyzable precursors thereof,

35 R<sup>3</sup> is an electron withdrawing group,

40 Y equals the number of atoms necessary to form an indole ring or a quinoline ring containing either hydrogen or a COOH group in the 2-position,

45 L is a ligand, and

50 M is a divalent or trivalent coordinate metal ion.

The pigments of this invention can be readily formulated with a polymeric binder to provide toner and developer particles having a controlled and predetermined size and size distribution and excellent triboelectric properties. These toners contribute to the formation of electrostatographic cyan color images having improved color and hue with minimum unwanted absorption outside of the cyan region of the spectrum thereby enabling the production of more faithful color reproductions of colored originals or even an enhancement of such originals.

The present invention also provides a process for preparing a cyan toner composition. The process comprises a first step of dispersing a concentrate containing the cyan pigment described hereinabove and a toner polymer material into an organic solvent which dissolves said polymer material and may or may not dis-

55 solve said pigment, but is immiscible with water to form an oil phase. A second step comprises mixing the oil phase under high shear mixing conditions with an aqueous phase containing a colloidal stabilizer to form a suspension of said oil phase in said aqueous phase. A third step comprises removing the solvent from said suspended oil phase. A fourth step comprises separating solidified particles of polymer/pigment mixture from said aqueous phase.

60 These and other features and advantages of the present invention will be better understood taken in conjunction with the following detailed description and claims.

## DETAILED DESCRIPTION

The cyan pigments represented by formulas 1 and 2 above are the metal coordination complexes of 6-heterocycloazo-3-pyridinol molecules having the structure of Formula 3:



wherein R, R<sup>1</sup>, R<sup>2</sup>, R<sup>3</sup> and Y are as set forth above.

The pigments may be in the form of 1:1 complexes having the structure of Formula 1 wherein L is a ligand capable of satisfying the coordination number of the metal. Preferred ligand groups include H<sub>2</sub>O, Cl, ammonia, acetate, pyridine or a second azo dye molecule. In a more preferred embodiment, these pigments are 2:1 complexes having the structure of Formula 2 (Formula 1 where L is a second identical tridentate dye moiety), because these latter pigments are generally more stable complexes.

M in Formulas 1 and 2 above is a divalent or trivalent metal ion which will complex with azo dye moieties having the structure of Formula 3. Such metal ions include Zinc II, Nickel II, Copper II, Cobalt II, and Cobalt III. Particularly good pigments are obtained where M is a divalent nickel ion.

The metallization reaction can be carried out in a single step process by reacting about 1 mole of a metal donating compound with about 1 mole of the appropriate azo compound to yield 1:1 complexes having the structure of Formula 1, or by reacting about 1 mole of the metal donating compound with about 2 moles of the appropriate azo compound to yield 2:1 complexes having the structure of Formula 2. Suitable metal donating compounds which may be used as the source of metal ions are metal salts including sulfates, acetates, nitrates and halides as well as complex salts such as metal amine salts or metal alkali salts of carboxylic acids or amino acids. The reaction takes place in a suitable solvent medium, for example, water, lower alkyl alcohol, formamide, glycol ethers, pyridine and the like, the choice of solvent being a function of the solubility of the reactants therein. Reaction temperatures may range from about 20° C. up to about 100° C. depending upon the ease of metallization of the particular diazo starting compound.

Monoazo dyes having the structure of Formula 3 may be prepared by generally well known diazotization and coupling methods using the appropriate reactants. The preferred method involves the diazotization of the fused ring heterocyclic compound, e.g., 8-aminoquinoline-5-sulfonamide or 5-nitro-8-aminoquinoline, using a mineral acid such as hydrochloric acid or trifluoroacetic acid and a source of nitrous acid such as sodium nitrite or isopentyl nitrite. The subsequent coupling of the diazonium salt with the appropriate 3-pyridinol compound, e.g., 2-amino-3-hydroxypyridine, is then carried

out according to known methods in an acid to alkaline medium and at temperatures generally below about 10° C.

In the more preferred embodiment of this invention, R<sup>2</sup> in the above formulas is selected from the group consisting of hydrogen, Cl, Br, SO<sub>2</sub>C<sub>6</sub>H<sub>5</sub>, SO<sub>2</sub>NH<sub>2</sub>, and SO<sub>2</sub>C<sub>6</sub>H<sub>4</sub>X where X is para-C<sub>1</sub> to C<sub>6</sub> alkyl, para-SO<sub>2</sub>CH<sub>3</sub>, para-OH, meta-SO<sub>2</sub>NH<sub>2</sub> or meta-SO<sub>2</sub>NHCH(CH<sub>3</sub>)<sub>2</sub>.

3. 10 In another preferred embodiment, electron withdrawing group R<sup>3</sup> is selected from the group consisting of NO<sub>2</sub> and SO<sub>2</sub>Z where Z is NH<sub>2</sub>, alkyl or alkoxy having from 1 to 12 carbon atoms and aryl or aryloxy having from 6 to about 10 carbon atoms.

15 15 The most preferred cyan pigments for use in manufacturing the toner and developer compositions of this invention are those of Formula 2 above wherein R is NH<sub>2</sub>, R<sup>1</sup> is hydrogen or CH<sub>3</sub>, R<sup>2</sup> is hydrogen or SO<sub>2</sub>C<sub>6</sub>H<sub>4</sub>X, where X is as defined above, R<sup>3</sup> is NO<sub>2</sub> and M is divalent nickel. These compounds generally absorb within the spectral range of from about 500-750 nm.

20 20 These and other dyes and dye complexes which may be used as precursor materials for the preparation of pigment in accordance with this invention are generally disclosed in U.S. Pat. No. 4,419,435, the complete disclosure of which is incorporated herein by reference.

25 25 Toner materials may be prepared in accordance with this invention by combining the pigment with a suitable polymer binder material such that the toner contains from about 2 to about 20% by weight of the pigment, more preferably from about 1 to 10% by weight, most preferably about 5% by weight.

30 30 The toner particles can comprise any fixable polymer which has the physical properties required for a dry electrostatographic toner. By fixable is meant simply that the toner particles can be fixed or adhered to a receiving sheet such as paper or plastic. Useful toners are often thermally fusible and fixable to the receiving sheet. However, toners which are otherwise fixable, such as solvent-fixable, pressure-fixable or self-fixable, can be prepared in accordance with the invention. These fixing techniques and toners suitable for them are well-known in the art.

35 35 40 45 50 55 55 60 65 Suitable polymers which may be used as binder materials in toners include, for example, olefin homopolymers and copolymers, such as polyethylene, polypropylene, polyisobutylene, and polyisopentylene; polyfluoroolefins such as polytetrafluoroethylene; polyamides such as polyhexamethylene adipamide, polyhexamethylene sebacamide and polycaprolactam; acrylic resins, such as polymethylmethacrylate, polyacrylonitrile, polymethylacrylate, polyethylmethacrylate and styrene-methylmethacrylate or ethylene-methyl acrylate copolymers, ethylene-methyl acrylate copolymers, ethylene-ethyl methacrylate copolymers, polystyrene and copolymers of styrene with unsaturated monomers mentioned above; cellulose derivatives, such as cellulose acetate, cellulose acetate butyrate, cellulose propionate, cellulose acetate propionate and ethyl cellulose; polyesters; polycarbonates; polyvinyl resins such as polyvinyl chloride and polyvinyl acetate, polyvinyl butyral, polyvinyl alcohol, polyvinyl acetal, ethylene-vinyl acetate copolymers, ethylene-vinyl alcohol copolymers and ethylene-allyl copolymers such as ethylene-allyl alcohol copolymers, ethylene-allyl acetone copolymers, ethylene-allyl benzene copolymers, ethy-

lene-allyl ether copolymers, ethylene-acrylic copolymers; and polyoxymethylene.

More preferred polymers for use as binder materials in toners include vinyl polymers, such as homopolymers and copolymers of styrene and condensation polymers such as polyesters and copolyesters. Especially useful toners are styrene polymers of from 40 to 100 percent by weight of styrene or styrene homologs and from 0 to 60 percent by weight of one or more lower alkyl acrylates or methacrylates. Fusible styrene-acrylic copolymers which are covalently lightly cross-linked with a divinyl compound such as divinylbenzene are useful, such as disclosed in Jadwin et al. U.S. Pat. No. Re. 31,072. Also especially useful are polyesters of aromatic dicarboxylic acids with one or more aliphatic diols, such as polyesters of isophthalic or terephthalic acid with diols such as ethylene glycol, cyclohexane dimethanol and bisphenols. Examples are disclosed in the above mentioned patent to Jadwin et al.

Fusible toner particles prepared according to this invention can have fusing temperatures in the range from about 50° C. to 200° C. so they can readily be fused to paper receiving sheets. Preferred toners fuse in the range of from about 65° C. to 120° C. If the toner transfer is made to receiving sheets which can withstand higher temperatures, polymers of higher fusing temperatures can be used.

Toner particles having the requisite particle size of about 0.1 to about 100 microns, more preferably from about 1 to about 30 microns, most preferably from about 2 to about 20 microns, can be prepared by techniques known in the art such as by hot melting a mixture of binder resin, pigment and any other addenda included in the composition, and grinding and screening the resultant bulk polymer composition. Other known techniques involve the suspension polymerization of monomers used to make the toner binder mixed with colorant and recovery of the suspended polymer particles, or the solvent/non-solvent method wherein a polymer and colorant are dissolved in solvent and the polymer/colorant mixture is caused to precipitate from the solvent by the addition of another solvent which is miscible with the first solvent but in which the polymer phase is non-soluble.

A particular advantage of the pigments of this invention is that they can be formulated into toner materials using evaporative limited coalescence procedures analogous to those disclosed in U.S. Pat. Nos. 4,833,060, 4,835,084 and 4,965,131, the complete disclosure of which patents is incorporated herein by reference. These processes provide toner particles of the requisite size and also of very narrow particle size distribution which is a very important characteristic for toner used in color electrophotography.

In accordance with a preferred procedure known as the polymer suspension method, a melt color concentrate may first be formed by hot milling an approximately 1:1 mixture of pigment and relatively high glass transition temperature polymer material, optionally containing minor quantities of a wax material. This mixture forms a brittle pigment concentrate upon cooling. This concentrate and additional binder polymer are then dissolved in a suitable solvent to form an oil phase. If the pigment is not completely soluble in the oil phase, the oil phase may also contain a suspension stabilizer to keep the pigment in suspension as it disperses in the oil phase.

Instead of first forming a pigment concentrate as described above, pigment particles can be simply ball milled with an organic solvent which also contains a minor amount of a pigment suspension stabilizer to form a pigment suspension, and this suspension may then be combined with binder polymer and additional solvent to form the oil phase.

Useful solvents for use in preparing the oil phase include those that dissolve the polymer and which are also immiscible with water including, for example, chloromethane, dichloromethane, ethyl acetate, vinyl chloromethane, vinyl chloride, methyl ethyl ketone, trichloromethane, carbon tetrachloride, ethylene chloride, trichloroethane, toluene, xylene, cyclohexanone, 2-nitropropane and the like.

The concentration of the polymer components in the solution may generally range from about 5 to about 30% by weight and the concentration of the pigment generally ranges from about 2 to about 15% by weight.

This solution is then introduced under high shear mixing conditions into an aqueous solution containing a solid colloidal stabilizing agent which may be finely divided silica as disclosed U.S. Pat. No. 4,833,060, or which may be a finely divided suspension of an interpolymer of styrene, 2-hydroxyethyl methacrylate, methacrylic acid, ethylene dimethacrylate, and optionally butyl methacrylate as disclosed in U.S. Pat. No. 4,965,131. The solvent is then caused to evaporate by heating the mixture under agitation, during which time the stabilizer present in the aqueous phase tends to limit the coalescence of the suspended polymer particles as they precipitate from the aqueous phase, thereby resulting in colored toner particles having the requisite particle size distribution.

The quantities of the various ingredients and their relationship to each other can vary over wide ranges. It has generally been found that the ratio of the polymer to the solvent should vary in an amount of from about 1 to about 80 percent by weight of combined weight of polymer and solvent and that the combined weight of the polymer in the solvent should vary with respect to the quantity of water employed in an amount of from about 25 to about 50 percent by weight. Also the size and quantity of the solid colloidal stabilizer depends upon the size of the particles of the stabilizer and also upon the size of the polymer particles desired. Thus, as the size of the polymer/solvent droplets are made smaller by high shear agitation, the quantity of solid colloidal stabilizer is varied to prevent uncontrolled coalescence of the droplets in order to achieve uniform size and narrow size distribution in the polymer particles that result.

Polymer particles having average diameters in the range of about 0.1 micron to about 100 microns, often from about 2 microns to about 20 microns can be prepared in accordance with the process of this invention. Such particles have a very narrow size distribution. Their coefficients of variation (ratio of the standard deviation to the average diameter) are normally in the range of about 15 to 35%.

Toner particles prepared in accordance with this invention can simply comprise the colored polymeric particles, but it is often desirable to incorporate addenda in the toner such as waxes, release agents, charge control agents and other toner addenda well known in the art.

Charge control agents suitable for use in toners are disclosed, for example, in U.S. Pat. Nos. 3,893,935;

4,079,014; 4,323,634; 4,812,381 and 5,075,190, as well as British Patent Nos. 1,501,065 and 1,420,839. Charge control agents are generally employed in small quantities such as from about 0.1 to about 3 weight percent, and preferably from about 0.2 to about 1.5 weight percent, based on the weight of the toner.

Toners prepared in accordance with this invention can be mixed with a carrier. The carriers which can be used to form suitable developer compositions can be selected from a variety of materials. Such materials include carrier core particles and core particles overcoated with a thin layer of film-forming resin.

The carrier core materials can comprise conductive, non-conductive, magnetic, or non-magnetic materials, such as disclosed for example, in U.S. Pat. Nos. 3,850,663 and 3,970,571. Especially useful in magnetic brush development schemes are iron particles such as porous iron particles having oxidized surfaces, steel particles, and other "hard" or "soft" ferromagnetic materials such as gamma ferric oxides or ferrites, including ferrites of barium, strontium, lead, magnesium, or aluminum. Such materials are disclosed in, U.S. Pat. Nos. 4,042,518, 4,478,925 and 4,546,060.

As noted above, the carrier particles can be overcoated with a thin layer of a film-forming resin for the purpose of establishing the correct triboelectric relationship and charge level with the toner employed. Examples of suitable resins are described in U.S. Pat. Nos. 3,547,822; 3,632,512; 3,795,618; 3,898,170; 4,545,060; 4,478,925; 4,076,857; and 3,970,571.

A typical developer composition containing the above-described toner and a carrier generally comprises from about 1 to 20 percent by weight of particulate toner particles and from about 80 to about 99 percent by weight of carrier particles. Usually, the carrier particles are larger than the toner particles. Conventional carrier particles have a particle size on the order of from about 20 to about 1200 microns, generally about 30-300 microns.

Alternatively, the toners of the present invention can be used in a single component developer, i.e., with no carrier particles, such as a toner comprising non-magnetic, insulative toner particles of an insulating binder resin as matrix containing the above described cyan pigment and optimally a charge control agent.

As stated above, the cyan toner prepared in accordance with this invention is adapted for use in a full color electrostatographic process along with complementary magenta, yellow and, optionally, black toners.

Illustrative of magenta toners are those containing 2,9-dimethyl substituted quinacridone; an anthraquinone dye identified in the Color Index as CI 60710, CI Dispersed Red 15; a diazo dye identified in the Color Index as CI 26050, CI Solvent Red 19; a diazo pigment identified in the Color Index as Pigment Red 122, and like known materials. Especially preferred magenta toners are those based on the 6-arylazo-3-pyridinol pigments as disclosed in applicants copending application Ser. No. 07/888,698, filed in the United States Patent and Trademark Office on even date herewith and entitled "Electrostatographic Toner Containing Magenta Pigment".

Illustrative of yellow toners include those containing permanent yellow FGL, Color Index Pigment Yellow 97, one of the preferred yellow materials which is prepared commercially by diazotization of 2,5 dimethoxy aniline-4-sulfonanilide, followed by coupling with 4-chloro-2,5 dimethoxy-acetanilide; diarylide yellow 3,3-

dichlorobenzidene aceto-acetanilide, a monoazo dye identified in the Color Index as CI 12700, CI Solvent Yellow 16; a nitrophenylaminesulfonamide identified in the Color Index as Foron Yellow Se-GLF, CI Dispersed Yellow 33; and the like. Especially preferred yellow toners are those based on the yellow diazo pigments as disclosed in applicant's copending application Ser. No. 07/888,696, filed in the United States Patent and Trademark Office on even date herewith and entitled "Electrostatographic Toner Containing Yellow Pigment".

Carbon black provides a particularly useful colorant for the optional black toner. The black toner may be a non-magnetic toner used as a monocomponent developer, or it may be a magnetic toner, e.g., containing magnetic material, or it may be used in the form of a two component magnetic developer with associated carrier particles.

The following examples are illustrative of the invention:

#### EXAMPLE 1

This example describes the preparation of a representative pigment complex having the structure of Formula 2 above wherein R is NH<sub>2</sub>, R<sup>1</sup> and R<sup>2</sup> are each hydrogen, R<sup>3</sup> is NO<sub>2</sub>, M is Ni II and Y=3 carbon atoms.

##### a) Preparation of 5-Nitro-8-Aminoquinoline Intermediate

8-Aminoquinoline was added portionwise over 10 minutes to a solution of acetic anhydride (40 g, 0.39M) and acetic acid (400 ml) while stirring at room temperature. The mixture was allowed to stir for one hour and then poured into ice water. The mixture was then made basic by the addition of 40% sodium hydroxide solution. The product was removed and dried at 40° C. for 12 hours to yield brown yellow crystals (91% yield).

Concentrated sulfuric acid (350 ml) was added to a 1000 ml 3-necked round bottomed flask and cooled to 5° C. 8-Acetamidoquinoline prepared as above (58.5 g, 0.314M) was added and stirred at 0° C. for 2 hours. Potassium nitrate (31.8 g, 0.315M) was added portionwise over a few minutes and the mixture was stirred for several hours. The mixture was poured into crushed ice to give a brown-yellow precipitate (55 g) in 76% yield.

5-Nitro-8-acetamidoquinoline prepared as above, (15 g, 64.9 mmol) was dissolved in tetrahydrofuran (75 ml) and treated with 40% hydrochloric acid (300 ml). The mixture was held at 80° C. for 3.5 hours and then allowed to cool. Tetrahydrofuran was removed under reduced pressure and the residual liquid was treated with saturated sodium bicarbonate solution until a neutral solution was obtained. The precipitate was removed by filtration to give 5-nitro-8-aminoquinoline (10 g).

##### b) Diazotization/Coupling Reaction

5-Nitro-8-Aminoquinoline prepared as above (15.7 g, 83.1 mmol) was dissolved in trifluoroacetic acid at 0° C. and treated with isopentyl nitrite (10.8 g., 92.3 mmol). The resulting mixture was added dropwise to a solution of 2-amino-3-hydroxypyridine (27.4 g, 249 mmol) and sodium acetate (800 g) in methanol at 0° C. and stirred for 30 minutes. Much of the methanol was removed by evaporation and the precipitate was removed by filtration. The solid was washed with a minimum amount of cold methanol to yield 9.7 g of product. Additionally, the filtrate was treated with saturated sodium bicarbonate and the organic phase was extracted with ethyl

acetate and ether from which phase a further 5.5 g product was obtained (totaling 15.2 g, 19.7% yield).

### c) Formation of Metal Complex

The product of step (b) above was added to methanol (1000 ml) and mixed with dimethyl formamide (400 ml) and water (50 ml) to obtain a solution. Nickelous acetate tetrahydrate was added (14.6 g, 58 mmol) and the reaction was allowed to stir overnight. The solvent was removed under reduced pressure to provide 17.1 g (40.3% yield) of the final 2:1 diazo metal complexed cyan pigment.

### EXAMPLE 2

This example describes a method for preparing colored toner particles using the cyan pigment prepared in Example 1 as a colorant.

### a) Preparation of Pigment Concentrate

A melt concentrate was prepared by mixing on a two roll mill at about 130° C. a 1:1 mixture of a finely ground pigment prepared according to Example 1 and a high molecular weight copolymer of styrene and butyl acrylate marketed by Goodyear under the trade designation PLIOTONE 4003. The concentrate composition also contained about 5% by weight of a hydroxy-terminated polyethylene wax added as a plasticizer. After cooling, the mass was comminuted to provide brittle chunks of pigment concentrate.

### b) Preparation of Pigment Oil Phase

To 14.27 g of ethyl acetate were added 6.32 g of the concentrate prepared in part (a) above. This mixture was stirred until the polymer was dissolved. While stirring, 4.40 g of a styrene/butyl acrylate addition copolymer (sold by Hercules as PICCOTONER 1221) and 0.012 g of tetradecylpyridinium tetraphenylborate (charge control agent) were added and stirring continued until the added components were uniformly dispersed or dissolved in the solvent.

### c) Preparation of Toner

24 g of the pigment oil phase prepared in part (b) above was dispersed using a high shear mixer into 119 ml of an aqueous pH 10 buffer solution also containing 45 2 grams of a latex suspension of a sub-micron size colloidal stabilizer based on an interpolymer of 8% by weight of styrene, 50% by weight of butyl methacrylate, 30% by weight of 2-hydroxyethyl methacrylate, 5% by weight of methacrylic acid and 7% by weight of ethyl 50 dimethacrylate.

The aqueous phase and organic phase were then homogenized using a Microfluidics Model M110F operating at 8100 psig. After homogenization, the ethyl acetate was removed by evaporation under a nitrogen stream with gentle mechanical stirring. 55

Coarse material was removed by filtration through a 50 micron screen and the toner particles were isolated by vacuum filtration. The toner particles were then washed thoroughly with distilled water and dried. The particles had an average particle diameter of about 6 microns with a particle size distribution range of about 2 to 10 microns.

### EXAMPLE 3

This example illustrates an alternative process for preparing colored toner particles using pigment of Example 1 as a colorant wherein the pigment oil phase is

prepared without first forming a concentrate as in Example 2.

10 g of the pigment of Example 1, 2 g of a pigment dispersant (marketed as ELVACITE™ AB1010 by Du Pont Corporation) and 100 g of ethyl acetate were mixed using a ball-mill until a fine suspension of the pigment in the solvent was obtained. 6.62 g of this suspension, 4.4 g of PICCOTONER 1221 binder and 0.012 g of tetradecylpyridinium tetraphenylborate charge agent were added to an additional 13.9 g of ethyl acetate and the mixture was stirred until the polymer and charge agent were dissolved.

Toner was then prepared by the polymer suspension process by dispersing 24.0 g of this oil phase into an aqueous phase exactly as set forth in part (c) of Example 2.

#### EXAMPLE 4

The toner material prepared in Example 3 was formulated into an electrostatographic developer as follows: 6 parts by weight of the toner particles of Example 3 were mixed with 94 parts by weight of a hard ferrite carrier coated with 1 pph of polyvinylidene fluoride and the mixture was shaken in a jar. The triboelectric properties of the toner were then evaluated on a magnetic brush development system. The initial positive triboelectric charge (charge-to-mass of toner) on the brush was measured at +86 microcoulombs per gram of toner. After 5 minutes of exercise on the brush, the charge was +69 microcoulombs per gram of toner.

The toner was transferred to a receiver sheet using a 300 volt bias at 22.8% relative humidity (RH). After heat fusing on the receiver, the transferred toner had a visible cyan spectrum which showed maximum absorbance at 664 nm.

Similar cyan pigments according to Formula 1 and Formula 2 are obtainable with analogous starting materials according to Formula 3, which may be formed into cyan toners, in accordance with the applicable procedures illustrated in Examples 1 through 4 hereinabove.

While the invention has been described in detail with reference to certain preferred embodiments, it will be understood that variations may be made by those skilled in the art without departing from the spirit and scope of the invention.

**What is claimed is:**

1. A dry, particulate electrostatographic toner composition comprising a binder polymer having mixed therewith a cyan pigment having a structure selected from the group consisting of:



and



wherein:

R is selected from the group consisting of OH and 20  
NH<sub>2</sub>;

R<sup>1</sup> is selected from the group consisting of hydrogen and C<sub>1</sub> to C<sub>6</sub> alkyl;

R<sup>2</sup> is selected from the group consisting of hydrogen, an alkyl group having from 1 to about 6 carbon atoms, acyl, aryl, aralkyl, alkylsulfonyl, amino, alkoxy, halogen, morpholino, phenylsulfamoyl, sulfonamido, sulfamoyl, carboxy and sulfo and hydrolyzable precursors thereof;

R<sup>3</sup> is an electron withdrawing group;

Y equals the number of atoms necessary to form an indole ring or a quinoline ring containing either hydrogen or a COOH group in the 2-position;

L is a ligand; and

M is a divalent or trivalent coordinate metal ion; said toner having an average particle size within the range of from about 0.1 to about 100 microns.

2. The toner of claim 1 wherein R<sup>2</sup> is selected from the group consisting of hydrogen, Cl, Br, SO<sub>2</sub>C<sub>6</sub>H<sub>5</sub>, SO<sub>2</sub>NH<sub>2</sub> and SO<sub>2</sub>C<sub>6</sub>H<sub>4</sub>X where X is para-C<sub>1</sub> to C<sub>6</sub> alkyl, para-SO<sub>2</sub>CH<sub>3</sub>, para-OH, meta-SO<sub>2</sub>NH<sub>2</sub>, or meta-SO<sub>2</sub>NHCH(CH<sub>3</sub>)<sub>2</sub>.

3. The toner of claim 1 wherein R<sup>3</sup> is selected from the group consisting of NO<sub>2</sub> and SO<sub>2</sub>Z, where Z is NH<sub>2</sub>, alkyl or alkoxy having from 1 to about 12 carbon atoms 45

and aryl or aryloxy having from 6 to about 10 carbon atoms.

4. The toner composition of claim 2 wherein R is NH<sub>2</sub>, R<sup>1</sup> is hydrogen or CH<sub>3</sub>, and R<sup>2</sup> is hydrogen or SO<sub>2</sub>C<sub>6</sub>H<sub>4</sub>X.

5. The toner composition of claim 4 wherein R<sup>3</sup> is NO<sub>2</sub>.

6. The toner composition of claim 1 wherein M is divalent nickel.

10 7. The toner composition of claim 1 wherein Y forms a quinoline ring.

8. The toner composition of claim 1 wherein said pigment has structure (b).

15 9. The toner composition of claim 8 wherein R is NH<sub>2</sub>, R<sup>1</sup> is hydrogen or CH<sub>3</sub>, and R<sup>2</sup> is hydrogen or SO<sub>2</sub>C<sub>6</sub>H<sub>4</sub>X where X is para-C<sub>1</sub> to C<sub>6</sub> alkyl, para-SO<sub>2</sub>CH<sub>3</sub>, para-OH, meta-SO<sub>2</sub>NH<sub>2</sub>, or meta-SO<sub>2</sub>NHCH(CH<sub>3</sub>)<sub>2</sub>.

10. The toner composition of claim 9 wherein R<sup>3</sup> is NO<sub>2</sub>.

11. The toner composition of claim 9 wherein Y forms a quinoline ring.

12. The toner composition of claim 10 wherein M is divalent nickel.

13. The toner composition of claim 8 wherein R<sup>1</sup> and R<sup>2</sup> are hydrogen, R<sup>3</sup> is NO<sub>2</sub>, Y forms a quinoline ring and M is divalent nickel.

14. The toner composition of claim 1 containing from 30 about 2 to about 20% by weight of said pigment.

15. The toner composition of claim 14 wherein said binder polymer is a copolymer of styrene with up to about 60% by weight of one or more lower alkyl acrylates or methacrylates.

16. The toner composition of claim 14 wherein said toner has an average particle size within the range of about 2 to about 20 microns.

17. A developer composition comprising a mixture of carrier particles and from about 1 to about 20% by weight of the toner composition of claim 1.

18. The toner composition of claim 1 wherein L is selected from the group consisting of H<sub>2</sub>O, Cl, ammonia, acetate and pyridine.

\* \* \* \* \*